

## UNITED STATES PATENT OFFICE

HELLMUT FISCHER, OF BERLIN-SIEMENSTADT, GERMANY, ASSIGNOR, BY MESNE ASSIGNMENTS, TO METAL & THERMIT CORPORATION, OF NEW YORK, N. Y., A CORPORATION OF NEW JERSEY

PROCESS FOR THE PRODUCTION OF BERYLLIUM ALLOYS, IN PARTICULAR THOSE WITH A HIGH BERYLLIUM CONTENT BY MEANS OF FUSED LIQUID ELECTROLYSIS

No Drawing. Application filed May 22, 1929, Serial No. 365,240, and in Germany November 13, 1928.

The production of beryllium alloys having a high beryllium content presents in practice considerable difficulties. The melting together of the beryllium with the alloy metals 5 is inadvisable for the reason that the beryllium easily burns away, and furthermore with such a process almost all the materials commonly used for the crucibles are too strongly attacked. Such a process would also take 10 much time as beryllium in a pure state dissolves but exceedingly slowly in other molten metals.

It has already been sought to produce beryllium alloys by means of fused liquid electrolysis. In this process the metals to be alloyed with beryllium have mostly been used in the molten state as cathodes. The result has generally been very non-homogenous alloys, as the diffusion of the beryllium in the other 20 molten metals is not sufficient to penetrate the outer layers which are saturated with beryllium and which can take up no more beryllium. It has, furthermore, already been proposed to produce beryllium alloys by adding 25 to a fused mass suitable for the electrolytic separation of beryllium, a salt of the other metals to be alloyed. This process is, however, technically difficult to carry out for the reason that the most suitable salts for the 30 process are generally hard to obtain.

These disadvantages of known processes are obviated by the present invention, according to which the metal to be alloyed with the beryllium is introduced by anodic solution 35 into the fused mass. During this procedure, the temperature of the fused mass is kept below the melting point of the metal to be alloyed.

It is particularly important in making 40 such alloy with beryllium, to use metals which have a greater specific gravity than the fused mass being used and which is preferably formed by a mixture of fluorides of beryllium and of one or more alkali earth metals. If 45 one of the lighter metals is to be alloyed with the beryllium, the specific gravity of the melt may be reduced by the addition of alkali metal halides to the fused mass.

The new process is preferably carried out 50 in the following manner, viz:—by first pro-

ducing in a crucible the above-mentioned fused mass and then connecting the crucible or at least the bottom of the crucible as an anode, while one or more cathodes, if necessary, cooled, are introduced from above into the fused mass. The metal to be alloyed, which is used advantageously in finely divided form, such as a powder, chips or the like, and approximately in the quantity suited for the desired beryllium content of the alloy, 55 is introduced at definite intervals of time into the fused mass during electrolysis. The highest permissible limit for the quantity of the alloy metal to be added to the fused mass 60 varies according to the specific gravity of the alloy produced. As soon as this would become greater than that of the electrolyte the separation would in practice be made much more difficult as the regulus formed at the cathode would dissolve therefrom. For copper the conditions are, for example, such that a beryllium alloy up to 50% can be produced 65 without special difficulties.

The metal to be alloyed with beryllium, 70 when introduced into the fused mass sinks to the bottom in consequence of its greater specific gravity and is then anodically polarized and dissolved under the action of the electric current. In this way there is formed the fluoride of the metal in question which is 75 otherwise very difficult to obtain and from this, the metal is separated, together with the beryllium, which is also present as a fluoride in the fused mass, as a beryllium alloy.

The new process is also particularly suitable for obtaining preliminary alloys with high beryllium content which can be further worked with beryllium alloys of lower percentage content by a small quantity thereof 80 being added to a fused mass of the metal to 85 be alloyed.

This use of the new process has important practical advantages as compared with the customary use of pure beryllium obtained by fused liquid electrolysis, as the starting material for the production of beryllium alloys. In particular by the formation of the alloy 90 of beryllium according to the new process, a considerable reduction of the melting point 95 of the separated material takes place and with 100

it the production of finer and smoother reguli. In consequence of the reduction of the melting point the operation can be conducted at lower temperatures than with the separation of beryllium alone, so that there is a noticeable saving of energy and furthermore the losses due to the volatilization of the beryllium are considerably reduced.

*Examples of carrying out the process*

(1) To a fused mass consisting of beryllium-fluoride and alkaline earth fluorides and suitable for the separation per hour of 200 g. of pure beryllium, 10 g. of copper in the form 15 of chips or powder were added every fifteen minutes. An approximately 15% copper-beryllium alloy was obtained from this fused mass by subjecting it to electrolysis.

(2) To a fused mass yielding 150 g. of pure 20 beryllium per hour and containing the same constituents as before, 20 g. of nickel were added every fifteen minutes, and a 35% nickel-beryllium alloy was obtained by electrolysis.

(3) To a fused mass of the same composition as before and permitting of the production of 500 g. of beryllium per hour, 5 g. of powdered iron were added every fifteen minutes, and a 3% iron beryllium alloy obtained by electrolysis.

The new process can of course be used to obtain alloys of beryllium with two or more other metals, in particular heavy metals. As an example of this the production of copper-nickel-beryllium alloys may be given, which can be effected by the simultaneous use of the Examples 1 and 2.

I claim:—

1. The process of producing beryllium alloys which consists in introducing into a fused mass containing beryllium, a metal to be alloyed with beryllium, such metal being of a specific gravity greater than that of the fused mass, and subjecting the mass to electrolysis.

2. The process of producing beryllium alloys which consists in introducing into a fused mass containing beryllium, a metal to be alloyed with beryllium, such metal being of a specific gravity greater than that of the fused mass, and having a melting point higher than the temperature of the fused mass, and subjecting the mass to electrolysis.

3. A process according to claim 1, in which the metal to be alloyed with beryllium is introduced gradually in comminuted solid form.

4. A process according to claim 1, in which the fused mass contains halides of beryllium and of a metal of the alkaline earths.

5. A process according to claim 1, in which the fused mass contains beryllium fluoride and a fluoride of a metal of the alkaline earths.

6. A process according to claim 1, in which the specific gravity of the fused mass is

maintained above that of the resulting beryllium alloy.

7. A process according to claim 1, in which the temperature of the fused mass is maintained, during electrolysis, below the melting point of the metal to be alloyed with beryllium.

8. A process for the production of beryllium alloys comprising melting in a crucible of electrically conducting material a mixture of fluorides of beryllium and one or more metals of the alkaline earths, connecting the crucible to the positive terminal of a source of current and a metallic body dipping into the fused mass to the negative terminal of such source, adding to the same from time to time a predetermined quantity of finely divided particles of a metal of a greater specific gravity than the fused mass, and maintaining the fused mass during electrolysis at a temperature below the melting point of the added metal.

In testimony whereof I affix my signature.  
HELLMUT FISCHER.

90

95

100

105

110

115

120

125

130